

149

Patented Nov. 4, 1930

1,780,595

Re 370,870

## UNITED STATES PATENT OFFICE

RALPH E. LAWRENCE, OF WICKLIFFE, OHIO, ASSIGNOR TO THE GRASSELLI CHEMICAL COMPANY, OF CLEVELAND, OHIO, A CORPORATION OF DELAWARE

## INHIBITOR

No Drawing.

Application filed October 9, 1929. Serial No. 398,570.

This invention relates to processes of cleaning and pickling of metal articles by the action of acids thereon and is particularly directed to the use in the pickling and cleaning 5 baths of certain organic substances which I found to have the property of inhibiting the action of acids upon the metal itself, without in any substantial manner impairing its action upon the oxide, rust, scale, salts or other 10 undesirable incrustation which such operations are intended to remove from the metal.

I found that mustard oils, when added to dilute, non-oxidizing acids have these inhibiting properties. Mustard oils are generally 15 characterized by having the formula CSN—R, in which R is a hydrocarbon radical. Typical members of this group are allyl-mustard oil, phenyl mustard oil, tolyl-mustard oil, naphthyl mustard oil, etc. The 20 higher members of this class of substances, particularly those in which the hydrocarbon radical is of the aromatic series, are not very volatile and the small amounts needed to produce the inhibiting action in pickling and 25 cleaning baths is insufficient to produce any amount of obnoxious vapors which might preclude their use.

Pickling and metal cleaning operations involve commonly the use of dilute acids, such 30 as sulfuric, hydrochloric, acetic, etc., or aqueous solutions of acid sulfates and such baths are used for numerous purposes of which pickling in steel mills and cleaning of pipe lines are the most typical representatives. 35 The concentration and composition of the bath, the temperature at which it is used and other factors vary of course in the different processes, though the underlying principle comprises always the removal of the undesirable 40 incrustations by the action of the acid. The bare metal so obtained is then unavoidably subjected to the acid and attacked so that besides the desired cleaning effect there is also quite a detrimental corrosion of the 45 clean metal which evidences itself in the weakening of the article and unnecessary consumption of acid. It has recently been shown that certain substances have the property of inhibiting the action of the acid upon 50 the metal itself without impairing its action

upon the incrustation and that this action is specific upon the hydrogen ion and quite independent of the anion of the acid bath, which in other words means that an inhibitor found efficient with sulfuric acid will show similar 55 inhibiting action with hydrochloric, acetic, or other non-oxidizing acids.

My novel inhibitors comprising the mustard oils are likewise efficient with the various commonly used pickling and cleaning acids. The application of my invention to acid pickling and acid metal cleaning operations does not involve any substantial change in the baths and operation itself, except the addition of a small amount of inhibitors. 65 Less than  $\frac{1}{2}$  of 1% of a mustard oil added to an acid pickling or cleaning bath will to a large extent, if not entirely, prevent the attack of the metal under the conditions where all undesirable incrustations are removed. In some instances amounts of less than 0.1% are already efficient and sufficient for all practical purposes. The use of my inhibitors in such operations results in a marked saving of acid and produces well 75 cleaned articles free from pitting or brittleness, so commonly found in acid treated metallic articles.

Mustard oils being quite difficultly soluble in dilute acids it is essential to have the 80 same well distributed through the pickling and cleaning baths, and as these cannot be stirred efficiently I prefer to disperse my inhibitors through the bath by first dissolving them in strong acids or mix them with protective colloids, such as sulfite cellulose waste, molasses residues, sulfonated vegetable oils, wetting agents, etc., such mixtures or solutions when added to the dilute acids precipitate the inhibitor in finely divided form and 85 render them much more active.

The actual efficiency of an inhibitor depends in large scale operations upon a number of factors and is rather difficult to determine. It can, however, be determined 95 comparatively by laboratory tests involving the measurement of gas evolved from a given surface of a piece of metal, immersed in a dilute acid containing the inhibitor. The less gas is evolved in a given time the more ef- 100

149

ficient is the inhibitor. While pickling operations use acid concentrations of the order of magnitude of 5 to 10% and temperatures of 60-70° C., I found that for laboratory tests 5 a 34% sulfuric acid used at room temperature provides a very convenient medium for testing the efficiency of inhibitors. I add to such acid various amounts of the inhibitor, immerse a piece of steel or other metal in such 10 bath and measure the amount of gas evolved after various periods.

The results tabulated below show cc. of 15 gases evolved from pieces of black mild sheet steel having 8 square inches surface immersed in such a test bath:

| Amount of inhibitor added to the bath    | 0.1%          | 0.05%          | 0.005%   |
|------------------------------------------|---------------|----------------|----------|
| Hours of immersion.....                  | 1 2 6 20      | 1 2 6 20       | 1 2 6 20 |
| Allyl-mustard oil.....                   | 0 0 0 23      | 0 0 0 18       | 1 5 6 10 |
| Phenyl mustard oil.....                  | 6 7 10 40     | 3 10 20 200    | -----    |
| Tolyl mustard oil.....                   | 3 8 15 170    | 6 55 130 >350  | -----    |
| Naphthyl mustard oil.....                | 12 20 82 >350 | 14 25 160 >350 | -----    |
| Same dispersed in 60° sulfuric acid..... | 0 0 1 1       | 5 8 54 130     | -----    |

25 A blank test made under the same conditions but without an inhibitor gave considerable more than 350 cc. of gas after 6 hours immersion.

My novel inhibitors are conveniently furnished in the form of a solution, emulsion or admixture with a strong acid, a protective colloid, such as sulfite cellulose waste, molasses residue, etc., or with such diluting agent as desired and which will produce a complete 30 dispersion of the active ingredient throughout the acid bath. All the pickler and cleaner has to do is to add such a composition to his standard acid bath and proceed in substantially the same manner as without my inhibitor.

I claim:

1. In a process of pickling and cleaning metal articles which comprises subjecting said articles to an acid bath containing as the active pickling and cleaning ingredient a non-oxidizing acid, the step of inhibiting the action of said acid upon the metal by the incorporation into the acid of an inhibitor comprising a mustard oil.
2. In a process of pickling and cleaning metal articles which comprises subjecting said articles to an acid bath containing as the active pickling and cleaning ingredient a non-oxidizing acid, the step of inhibiting the action of said acid upon the metal by the incorporation into the acid of an inhibitor comprising a mustard oil in fine dispersion throughout said acid bath.
3. A composition of matter for pickling and cleaning metal articles comprising a dilute, non-oxidizing acid and a small amount of an inhibitor comprising a mustard oil.
4. A composition of matter for pickling 65 and cleaning metal articles comprising a

dilute, non-oxidizing acid and a small amount of an inhibitor comprising a mustard oil in fine distribution throughout the bath.

In testimony whereof, I affix my signature.

RALPH E. LAWRENCE.

70

75

80

85

90

95

100

105

110

115

120

125

130